

[54] **MOLYBDENUM-TITANIUM-ZIRCONIUM-ALUMINUM MASTER ALLOYS**

[75] Inventor: **Frederick H. Perfect**, Wyomissing, Pa.

[73] Assignee: **Reading Alloys, Inc.**, Robesonia, Pa.

[21] Appl. No.: **801,086**

[22] Filed: **May 27, 1977**

[51] Int. Cl.<sup>2</sup> ..... **C22C 21/00**

[52] U.S. Cl. ..... **75/134 F; 75/138; 75/175.5; 75/176**

[58] Field of Search ..... **75/138, 134 F, 176, 75/175.5; 148/32**

[56] **References Cited**

**U.S. PATENT DOCUMENTS**

3,725,054 4/1973 Perfect ..... 75/138

*Primary Examiner*—R. Dean

*Attorney, Agent, or Firm*—Howson & Howson

[57] **ABSTRACT**

This invention relates to molybdenum-titanium-zirconium-aluminum master alloys containing about 35 to 40 molybdenum, about 1 to 5% titanium, about 15 to 25% zirconium, balance aluminum and not more than about 0.004% nitrogen.

**3 Claims, No Drawings**

**MOLYBDENUM-TITANIUM-ZIRCONIUM-  
ALUMINUM MASTER ALLOYS**

**DESCRIPTION OF THE INVENTION**

Titanium base alloys such as the alloys 6Al-2Sn-4Zr-2Mo and 6Al-2Sn-4Zr-6Mo find use in the manufacture of certain aircraft. Heretofore, these titanium base alloys have been produced through the addition of a 45Al-55Mo master alloy and zirconium sponge to titanium base metal. However, it has been found that the resultant alloys may contain nitride inclusions thought to emanate from zirconium sponge. Hence, there is a need for zirconium containing master alloys for use in preparing the titanium base alloys described above. Master alloys thought to be useful in the manufacture of titanium alloys containing 30-45% Mo, 20-30% Zr, balance aluminum are described in USSR Pat. No. 297,695 cited in Chemical Abstracts, Volume 75-90831x. U.S. Pat. Nos. 3,625,676 and 3,725,054, disclose vanadium, aluminum, titanium and molybdenum, titanium, aluminum master alloys respectively.

According to this invention there is provided molybdenum-titanium-zirconium-aluminum master alloys containing from about 35 to about 40% molybdenum, from about 1 to about 5% titanium, from about 15 to about 25% zirconium, balance aluminum, said alloys containing not more than about 0.004% by weight, nitrogen and being suitable for use in making titanium base alloys.

The master alloys are produced by the aluminothermic reduction of the oxides of molybdenum, titanium, and zirconium with excess aluminum to metallic molybdenum, titanium and zirconium which combine with aluminum forming the desired master alloys. It has been found that master alloys having a composition described herein are homogenous, friable, substantially free of slag, and remarkably low in nitrogen content. In addition, the master alloys can be sized to  $\frac{1}{8}$  by 100 mesh without creating substantial quantities of pyrofornic fines, and combine readily with titanium sponge in this form.

The master alloys of this invention may be produced in any suitable apparatus. A preferred type of reaction vessel is a water-cooled copper vessel of the type described in "Metallothermic Reduction of Oxides in Water-Cooled Copper Furnaces", by F. H. Perfect, transactions of the Metallurgical Society of AIME, Volume 239, August 1967, pp. 1282-1286.

In producing the master alloys of this invention, oxides of molybdenum, titanium, and zirconium, are reduced to a relatively small size, and intimately mixed so that reaction will occur rapidly and uniformly throughout the charge on ignition. An excess of aluminum is used to produce the alloy. Ignition of the reaction mixture may be effected by heating the charge to above the melting point of aluminum by an electric arc, gas burners, hot metal bar, wire or the like.

Relatively pure molybdc oxide (molybdenum dioxide), containing 99 plus %  $\text{MoO}_3$ , or very pure calcium molybdate, may be used as the source of molybdenum.

It is preferred to use pigment grade titanium dioxide which analyzes 99 plus %  $\text{TiO}_2$  as the source of titanium. However, less pure  $\text{TiO}_2$ -containing material, such as native rutile, which analyzes about 96%  $\text{TiO}_2$ , and contains minor amounts of the oxides of Fe, Si, Zr, Cr, Al and Ca as well as S and P, as impurities, may be

employed. Commercial grade  $\text{TiO}_2$  is preferably since its use enhances the purity of the resulting master alloy.

Relatively pure zirconium oxide ( $\text{ZrO}_2$ ) or Baddeleyite containing 99 %  $\text{ZrO}_2$ , may be used as the source of zirconium.

The aluminum powder should be of the highest purity available commercially. Virgin aluminum powder analyzing an excess of 99% aluminum, is the preferred reducing agent and addition agent.

Due to natural variance in purity of the metal oxide and aluminum reactants, the proportion of the constituents rerequired to provide master alloys of a given composition will vary. For this reason, the respective amounts of materials used are expressed in terms of the composition of the desired alloy. As stated above, the amount of components should be so proportioned as to provide master alloys containing from about 35 to about 40% molybdenum, from about 1 to about 5% titanium,

from about 15 to about 25% zirconium, balance aluminum. The master alloys produced contain not more than about 0.004%, by weight, nitrogen, and incidental amounts of boron, carbon, iron, hydrogen, oxygen, phosphorus, silicon, and sulfur. Preferred master alloys

comprise from about 36 to about 39% molybdenum, from about 3 to about 5% titanium, from about 18 to about 22% zirconium, balance aluminum. A calcium aluminate slag is produced during the reaction, and the reaction is carried out in the presence of a molten flux

which dilutes the slag and renders it more fluid in order that the slag may be separated from the alloy. The flux must be capable of diluting the slag formed by the reaction to produce a less viscous slag which separates readily from the alloy. The fluorides and chlorides of

metals such as Ca, Na, and K, alone or in combination with other inorganic materials, are particularly suitable for forming slag-absorbing fluxes.

The amount of flux-forming agents employed should

be sufficient to provide an amount of molten flux capable of diluting the slag formed during oxide reduction to provide a less viscous slag which is readily separated from the metal. Preferably an excess of flux over that

needed to obtain the desired reduction in slag viscosity is used. The excess may be from about 0.5 to 2 times the weight of the slag formed in the process.

The resulting molybdenum-titanium-zirconium-aluminum master alloys are homogenous, relatively

void free and, as noted above, contain less than 0.004% nitrogen, by weight. Moreover, the master alloys of this

invention are clean, and free of gross nitride inclusions.

The master alloys can be reduced in particle size to 8 mesh or less to permit fluoroscopic examination. When

reduced to this size, the master alloys become relatively transparent to fluoroscopic inspection. Of course, reduction of the master alloy to 8 mesh or less, creates a hazard since many pyrofornic fines are produced. Hence,

the master alloy is typically reduced to  $\frac{1}{8}$  by 100 mesh, and in this form, may be blended with a titanium sponge in sufficient amounts to provide the desired titanium base alloys.

The master alloys can be reduced in particle size to 8 mesh or less to permit fluoroscopic examination. When

reduced to this size, the master alloys become relatively transparent to fluoroscopic inspection. Of course, reduction of the master alloy to 8 mesh or less, creates a hazard since many pyrofornic fines are produced. Hence,

the master alloy is typically reduced to  $\frac{1}{8}$  by 100 mesh, and in this form, may be blended with a titanium sponge in sufficient amounts to provide the desired titanium base alloys.

The following examples are illustrative of the invention:

**EXAMPLE I**

The materials in Table I were combined and mixed together:

Table I

| Ingredient         | Weight (lbs.) |
|--------------------|---------------|
| MoO <sub>3</sub>   | 77            |
| TiO <sub>2</sub>   | 10            |
| ZrO <sub>2</sub>   | 50            |
| Al                 | 108           |
| CaF <sub>2</sub>   | 25            |
| CaO                | 25            |
| NaClO <sub>3</sub> | 10            |

After mixing, the charge was placed in a crucible, ignited and allowed to run 50 to 55 seconds. Metal-slag separation was good, and the resultant alloy weighed 130 lbs. The analysis of the alloy is in Table II.

Table II

|    | Percent |
|----|---------|
| Mo | 39.66   |
| Ti | 4.77    |
| Zr | 20.64   |
| Al | 34.39   |
| N  | 0.004   |
| O  | 0.081   |

## EXAMPLE II

Following the procedure of Example I, an alloy was prepared from the mixture shown in Table III.

Table III

| Ingredient       | Weight (lbs.) |
|------------------|---------------|
| MoO <sub>3</sub> | 77            |
| TiO <sub>2</sub> | 10            |

10

Table III-continued

| Ingredient              | Weight (lbs.) |
|-------------------------|---------------|
| ZrO <sub>2</sub> (pure) | 50            |
| Al                      | 108           |
| CaF <sub>2</sub>        | 10            |
| CaO                     | 35            |
| NaClO <sub>3</sub>      | 10            |

The resulting alloy has the analysis shown in Table IV.

Table IV

|    | Percent |
|----|---------|
| Mo | 36.53   |
| Ti | 3.79    |
| Zr | 20.65   |
| Al | 38.6    |
| N  | 0.004   |
| O  | 0.082   |

Having thus described the invention,

What is claimed is:

1. A molybdenum-titanium-zirconium-aluminum master alloy comprising from about 35 to about 40% molybdenum, from about 1 to about 5% titanium, from about 15 to about 25% zirconium, balance aluminum, said alloy containing not more than about 0.004%, by weight, nitrogen.
2. The master alloy of claim 1 comprising from about 36 to about 39% molybdenum, about 3 to about 5% titanium, from about 18 to about 22% zirconium, balance aluminum.
3. The master alloy of claim 1 comprising about 39.6% molybdenum, 4.7% titanium, 20.6% zirconium, balance aluminum.

\* \* \* \* \*

30

25

35

40

45

50

55

60

65